

April 7, 1936.

R. P. RICHARDSON

DRAFTING OF COTTON AND LIKE FIBERS

2,036,886

Filed Dec. 20, 1934

2 Sheets-Sheet 1

Fig. 1.



Fig. 2.



Fig. 3.



Fig. 4.



Inventor:

Ralph Pillsbury Richardson

By *L. F. Nichols*  
Attorney

April 7, 1936.

R. P. RICHARDSON  
DRAFTING OF COTTON AND LIKE FIBERS

2,036,886

Filed Dec. 20, 1934

2 Sheets-Sheet 2



Inventor:

Ralph Pillsbury Richardson  
By *John F. Geiger*  
Attorneys

## UNITED STATES PATENT OFFICE

2,036,886

## DRAFTING OF COTTON AND LIKE FIBERS

Ralph Pilsbury Richardson, Bombay,  
British IndiaApplication December 20, 1934, Serial No. 758,497  
In Great Britain April 24, 1933

4 Claims. (Cl. 19—130)

My invention relates to improvements in the drafting of cotton and like staple fibers in the manufacture of yarn and thread.

One of the objects of my invention is to obviate the extravagance of drafting effort consequent upon the present day mode of drawing-frame doubling. In mill practice, a fixed draft roller setting interval obviously cannot select and draft fibers of greatly varying length in a positive manner. Much of the necessary draft therefore has unavoidably to depend upon the chance movement of the fibers of shorter length. Doubling as commonly practiced, which involves combining a plurality of ordinary card slivers, usually six in number, is, apart from its being the source of productive power of the system, generally believed to possess the virtue of minimizing the undesirable effects of the present haphazard method of chance fiber drafting.

Such doubling which involves presenting to the drafting rollers a relatively thick strand of fibers, results in an overcrowding of the effective nip of the rollers and thus less positive selectivity of the fibers.

My invention is based upon a new and comprehensive conception of the doubling and drafting functions and involves presenting a minimum number of fibers per unit roller nip length at each drafting stage. In consequence the drafting rollers are afforded the opportunity of directly selecting and withdrawing in a positive manner from the strand, at each draft zone, a greater number of fibers in any given interval of time than is at present possible in everyday standard practice.

The invention will be readily understood from the following description in conjunction with the accompanying drawings in which:

Figure 1 shows diagrammatically a layout or drafting system embodying the invention.

Figures 2, 3 and 4 are views of three guiding devices for use in the system shown in Figure 1 and,

Figure 5 is a perspective view of a suitable form of doffer and coiler mechanism while

Figure 6 shows the doffer employed.

Referring to Figure 1, 1 indicates the passage of the material through a revolving flat carding engine, the full width doffer web being divided into four part slivers of equal size and delivered at a. This is intended for the higher range of yarn counts; in the case of the lower yarn-count range six such part-slivers are employed. Means necessary for dividing the doffer web will be associated with the doffer and coiler mechanism and will be readily apparent to one versed in the art but one form of construction which may be employed is hereinafter indicated.

Eight of the part-slivers are then passed from b through the rollers of a drawing-frame 2 which

comprises four rollers from which the slivers emerge as a combined sliver as at c. If, however, the doffer web had been divided into six part-slivers, twelve of such slivers would be combined in the drawing-frame 2. Where so desired, as for example, in the event of processing finer or alternatively better quality yarns, a second passage of drawing-frame may be utilized. In this case eight or, in the case of initial division into six part-slivers, twelve of the slivers c are now passed through the rollers of a second drawing-frame 3 and combined into a single sliver designated e, three of which slivers are shown passing from f, through the rollers of a fly-frame or slubber 4 to be doubled into a single strand of g. The latter step is repeated from h in a second fly-frame or rover 5 and three of the strands i produced are shown passing from j through the rollers of a spinning frame 6 to be drafted and twisted into the single thread o of yarn at k.

The traversing guides 7, 8 and 9 shown in Figures 2, 3 and 4 are employed in conjunction with the fly-frames 4 and 5 and the spinning frame 6, respectively, and serve to guide the strands through the rollers at the frames 4, 5 and 6 while giving maximum width of ribbon without any possible overlapping of the three unit strands at each stage.

Any suitable mechanism may be employed for the division of the doffer web. For example, it will be apparent that doffer and coiler mechanism as are employed in the treatment of cotton waste may be utilized. One such known construction is shown in Figures 5 and 6.

The doffer 10, which is more particularly shown in Figure 6, is of the ordinary type and the fillet is also standard. The surface of the roller is however divided by leather bands of about  $\frac{3}{8}$  inch width or more or less, into four parts of equal area. Of course the number of leather dividers employed depends upon the number of part-webs into which the card is divided. Likewise the number of coiler and can mechanisms will also correspond to the number of part-slivers desired.

In operation the fleece is stripped by the comb (not shown) in the standard way and is divided by the leather bands 15 into four equal-size part webs covering the areas indicated by 14. Through the guides 11 the part-webs separately pass to coiler mechanisms 12 and are coiled in cans (not shown) placed on the base 13. It will be understood that instead of leather dividers steel blades, for example, could be employed in the manner known per se for dividing the doffer web.

In carrying out the invention, it is found that a closer setting is required between each pair of draft rollers and this closer setting allows the

rollers to select a greater number of fibres of correspondingly shorter length.

As has hereinbefore been pointed out the important feature of the present invention consists in presenting a minimum number of fibers per unit roller nip length at each successive draft stage. Technologically the ideal conditions, for maximum fiber selectivity with my invention, would be attained if the fleece or strand at each stage were one fiber thick and the fibers comprising the width of the fleece were lying parallel and closely side by side without any loss of roller-width and with no overlapping of the fibers. But in commercial mill practice this ideal is not attainable because (1) one width of carding engine has to serve a wide range of yarn counts, and (2) the number of fibers necessary to form any given count of yarn is, due to their varying quality, not necessarily the same in all cases.

For these reasons alone it is not practicable to prescribe for any given count of yarn or range of counts the number of part-slivers into which a given doffer web must be divided to give optimum result. For average practice in the case of the doffer web of a 37 inch carding engine, four equal size part-webs are employed for 70's counts of yarn and upwards. For counts of 30's to 70's a 40 inch card web is divided into five equal part-webs and for counts below 36's a 45 inch doffer web is divided into six equal part-webs.

In the tables below set forth specific data is given to show one possible scheme of draft according to the invention in comparison with a typical example of the standard practice now in vogue for the production of yarn of the type of 40's count specified.

#### Standard practice

| 40                                                                                   | Carding engine                                                                                                                  | Drawframe No. 1                                                                                                                    | Drawframe No. 2 |
|--------------------------------------------------------------------------------------|---------------------------------------------------------------------------------------------------------------------------------|------------------------------------------------------------------------------------------------------------------------------------|-----------------|
| 0.15 hank card sliver will contain approximately 25,200 fibers in its cross section. | 6 ends up, 6.2 draft, 0.155 hank drawing. These six slivers at back occupy 4", 4 1/4" at front.<br>R{Back=37800.<br>Front=5795. | 6 ends up, 6.5 draft, 0.169 hank finished sliver. These 6 slivers occupy 4" at back: 4 1/4" front.<br>R{Back=36750.<br>Front=5260. |                 |
| 45                                                                                   |                                                                                                                                 |                                                                                                                                    |                 |

#### My system

| 50 | Carding engine                                                                                                      | Drawframe No. 1                                                                                                                             | Drawframe No. 2                                                                                                                              |
|----|---------------------------------------------------------------------------------------------------------------------|---------------------------------------------------------------------------------------------------------------------------------------------|----------------------------------------------------------------------------------------------------------------------------------------------|
| 55 | 0.15 hank card sliver divided into five equal part slivers equal 0.75 hank sliver or 5,040 fibers in cross section. | 10 ends up, 7.2 draft, 0.54 hank sliver drawing. These 10 slivers occupy 4 1/2" at back and 4 3/4" at front.<br>R{Back=11200.<br>Front=1472 | 10 ends up, 7.8 draft, 0.42 hank finished sliver. These 10 slivers occupy 4 1/2" at back and 4 3/4" at front.<br>R{Back=15250.<br>Front=1888 |
| 60 |                                                                                                                     |                                                                                                                                             |                                                                                                                                              |

#### Standard practice

| 65 | Slubber                                                                                                                          | Intermediate                                                                                                     | Rover                                                                                                 | Spinning                                                                                      |
|----|----------------------------------------------------------------------------------------------------------------------------------|------------------------------------------------------------------------------------------------------------------|-------------------------------------------------------------------------------------------------------|-----------------------------------------------------------------------------------------------|
| 70 | 1 end up, 4.0 draft, 0.678 hank slubbing. This one sliver contains 22,360 fibers in 3/4" at back.<br>R{Back=29813.<br>Front=7440 | 2 ends up, 4.7 draft, 1.58 hank. These two slivers contain 11,200 fibers in 3/4".<br>R{Back=35840.<br>Front=7648 | 2 ends up, 5.7 draft, 4.60 hank roving. 4733 fibers contained in 1/2".<br>R{Back=38264.<br>Front=6720 | 1 end up, 9.0 draft, 40's counts 840 fibers contained in 1/2".<br>R{Back=16800.<br>Front=1880 |
| 75 |                                                                                                                                  |                                                                                                                  |                                                                                                       |                                                                                               |

#### My system

| Slubber                                                                                                                             | Intermediate                                                                       | Rover                                                                                                               | Spinning                                                                                                    |   |
|-------------------------------------------------------------------------------------------------------------------------------------|------------------------------------------------------------------------------------|---------------------------------------------------------------------------------------------------------------------|-------------------------------------------------------------------------------------------------------------|---|
| 3 ends up, 8.8 draft, 1.23 hank slubbing. These 3 ends at back occupy 7/8" and contain 26991 fibers.<br>R{Back=30847.<br>Front=3511 | Omitted. (As a consequence of this, the ratio R increases at the adjacent stages.) | 3 ends up, 11.0 draft, 4.5 hank roving. These 3 slivers contain 9216 fibers in 1/4".<br>R{Back=36864.<br>Front=3360 | 3 ends up, 27.0 draft, 40's counts. These 3 ends contain 2520 fibers in 3/4".<br>R{Back=16800.<br>Front=622 | 5 |

The value "R" given in the above tables relates to one specific example only and is by way of illustration. R is represented by the number of fibers per inch of length of roller nip or width of fleece employed. This fleece width is governed by the effective width of the strand guides employed (e.g., as in Figs. 2, 3 and 4) acting in conjunction with the top roller loading weights used to compress the fleece. The thickness of the fleece at each stage may be represented by the number of fibers which compose the fleece thickness. The quality of the particular cotton mentioned above is such that it requires 1666 such fibers lying parallel and closely side by side without overlapping to form a fleece one inch wide and one fiber thick, so that the thickness of the first drawing frame fleece shown with the present invention in the above table is approximately 6 3/4 fibers at presentation and .9 fiber thick at the emergent fleece. (The corresponding figures with the standard system shown are 22.7 and 3.5 fibers, respectively.)

In general mill practice, this fleece width-thickness relationship will unavoidably fluctuate greatly. But whereas the width of the fleece will be controlled within relatively narrow limits, the thickness of the fleece will vary greatly, depending upon the carding engine-cum-yarn count range relationship, the number of drafting stages and the amount of draft employed at each stage, the width of the fleece and the number of fibers contained in the fleece. It should be mentioned that 0.15 hank sliver represents the safe maximum limit of output of good quality sliver for 40's counts from a 40 inch carding engine with a 26 inch doffer running at 14 revolutions per minute. The formula employed for the calculation of the fiber number is

$$N = \frac{529}{W \cdot C}$$

where W is  $0.14 \times 10^{-6}$ , the weight of fiber and C is the count or hank of strand. N represents the number of fibers comprising a single strand. In the following table is given data relative to the cotton employed and yarn produced.

| Cotton quality                                                                                                          | Yarn quality                                                                             |
|-------------------------------------------------------------------------------------------------------------------------|------------------------------------------------------------------------------------------|
| Average fiber length—1.0 inch<br>Average fiber weight— $0.14 \times 10^{-6}$ ounce<br>Average fiber strength—0.14 ounce | Yarn counts—40's.<br>Lea strength in lbs.—40.                                            |
| Average fiber (ribbon) width— $0.8 \times 10^{-3}$ inch.                                                                | Turns per inch—25.3 or 40's counts.<br>Front roller speed $7/8$ dia., 140 revs. per min. |
|                                                                                                                         |                                                                                          |

The foregoing detailed description has been given for clearness of understanding only and no unnecessary limitation should be understood therefrom. For example the invention is applicable to all counts of carded and combed yarns.

Again the draft stages may vary with, for example, the quality of yarn to be produced. In the case of a good quality 20's yarn the following scheme may be adapted:—starting with a 5 hank of card sliver of 0.17, the drafts at the frames 2 and 3 (Figure 1) are 7.4 and 8.0 respectively followed by a slubber draft as at 4 of 9.0 with a final draft of 24 in the spinning machine as at 6.

10 I claim:—

1. A process of drafting cotton and like staple fibers which comprises dividing the full-width doffer web of a cotton revolving flat carding engine into from four to six equal size part-webs, according to the width of the doffer and the type of yarn required, combining the part-slivers from two such doffer webs by passage through drafting rollers of a drawing frame, so that the number of fibers per inch of width of the web on said 15 rollers will be maintained at a low value compared to standard practice, feeding three separately guided combined slivers from the drawing frame through a fly-frame to form a strand of rove and separately guiding three of such fine 20 rovings produced to a final spinning frame, wherein said rovings are combined and twisted 25 into the final strand of yarn.

2. A process of drafting cotton and like staple fibers which comprises dividing the full-width doffer web of a cotton revolving flat carding engine into from four to six equal size part-webs, according to the width of the doffer and the type of yarn required, combining the part-slivers from two such doffer webs by passage through drafting rollers of a drawing frame, so that the number of fibers per inch of width of the web on said 30 rollers will be maintained at a low value compared to standard practice, feeding three such combined slivers from the drawing frame through a fly-frame to form a strand of rove, passing three such strands of rove through a second fly-frame, and combining three of such fine rovings produced to a final spinning frame, wherein said rovings are 35 produced in a final spinning frame, wherein said 40

rovings are combined and twisted into the final strand of yarn.

3. A process of drafting cotton and like staple fibers which comprises dividing the full-width doffer web of a cotton revolving flat carding engine into from four to six equal size part-webs, according to the width of the doffer and the type of yarn required, combining a number of such part-webs equivalent to two such doffer webs by passage through a delivery of a drawing frame, 10 so that the number of fibers per inch of width of the web on said rollers will be maintained at a low value compared to standard practice, passing such a number of combined slivers through a second drawing frame delivery, feeding three separately guided combined slivers produced through a fly-frame to form a strand of rove, passing three separately guided rovings through a second fly-frame, and separately guiding three of such fine rovings produced to a final spinning frame, 20 wherein said rovings are combined and twisted into the final strand of yarn.

4. A process of drafting cotton and like staple fibers which comprises dividing the full-width doffer web of a cotton revolving flat carding engine into from four to six equal size part-webs, according to the width of the doffer and the type of yarn required, combining a number of such part-webs equivalent to two such doffer webs by passage through a delivery of a drawing frame, 25 so that the number of fibers per inch of width of the web on said rollers will be maintained at a low value compared to standard practice, passing such a number of combined slivers through a second drawing frame delivery, feeding three such 30 combined slivers produced through a fly-frame to form a strand or rove, passing three such strands of rove through a second fly-frame, and feeding three of such fine rovings produced to a final spinning frame, wherein said rovings are 35 combined and twisted into the final strand of yarn.

RALPH PILSBURY RICHARDSON.